# EUROPEAN PATENT SPECIFICATION

(11) **EP 2 708 616 B1**
(45) Date of publication and mention of the grant of the patent: **07.12.2016**
(21) Application number: 12782900.0
(22) Date of filing: 07.05.2012
(51) Int. Cl.: C23C 2/20, C23C 2/40

(54) **GAS WIPING DEVICE**
GASNITRIERUNGSVORRICHTUNG
DISPOSITIF D'ESSUYAGE AU GAZ

(30) Priority: 09.05.2011 JP 2011104089; 12.03.2012 JP 2012054183
(43) Date of publication of application: 19.03.2014
(73) Proprietor: Nippon Steel & Sumikin Engineering Co., Ltd., Tokyo 141-8604 (JP); NS Plant Designing Corporation, Fukuoka 804-0002 (JP)
(72) Inventor: WAKABAYASHI Hisamoto, Kitakyushu-shi, Fukuoka 804-8501 (JP); KATSUBE Makoto, Kitakyushu-shi, Fukuoka 804-8501 (JP); NISHIKAWA Hiroshi, Kitakyushu-shi, Fukuoka 804-0002 (JP)
(74) Representative: Wohlfahrt, Jan Günther
(86) International application number: PCT/JP2012/061644
(87) International publication number: WO 2012/153702

(56) References cited:
- JP-A- 1 290 755
- JP-A- 52 141 430
- JP-A- 2006 274 381
- JP-A- 2007 284 732
- JP-A- 2007 284 732
- JP-U- H03 125 058
- US-A- 3 977 359

## Description

### TECHNICAL FIELD

The present invention relates to a gas wiping device for adjusting the amount of molten metal for plating that becomes attached to a surface of a steel strip as the steel strip is continuously transported and immersed in a plating bath, by spraying gas onto the surface.

### BACKGROUND ART

When molten metal plating is performed by continuously immersing a steel strip in a molten metal plating bath, so-called gas wiping is generally performed, whereby gas is sprayed onto an unsolidified plated surface of the steel strip after immersion so as to adjust the amount of attached molten metal. For example, gas wiping devices with gas wiping nozzles are disposed on both sides of the continuously transported steel strip, and gas wiping is performed by blowing gas onto both sides of the steel strip.

The gas wiping nozzles have an elongated shape corresponding to the length of the steel strip in the width direction thereof. The steel strip is transported upward in front of the gas wiping nozzles while being immersed in the molten metal in the plating pot. The gas wiping nozzles have a slit-shaped gas outlet for blowing out the gas that extends along the width direction (longitudinal direction) of the steel strip. By spraying the gas out of the gas outlet onto the steel strip linearly across one end to the other in the width direction of the steel strip, the molten metal on the surface of the steel strip is removed in a desired manner, thus adjusting the amount of attached molten metal.

The gas wiping is associated with the problem of overcoating in which the amount of molten metal attached to the edges of the steel strip in the width direction becomes greater than at other portions, or splashing in which the molten metal removed by the gas is scattered at the edges. The problems of overcoating and splashing are caused by turbulence produced by the collision of the streams of gas discharged out of opposing gas wiping nozzles near the edges of the steel strip, for example.

In order to suppress overcoating at edges of a steel sheet while suppressing the noise and vibration during gas wiping, patent document 1 discloses a hollow gas wiping nozzle for use in hot dip galvanization of a steel plate to adjust the coating thickness. Patent document 2 discloses a coating apparatus for effecting a uniform coating of a molten metal which includes an air-knife means having a sliding shutter disposed within the nozzle at each end of the slot thereof.

In order to decrease the overcoating or splashing at the edges of the steel strip in the width direction, Patent Document 3 discloses a gas wiping device including a slit blocking mechanism for making the edge positions of the slit of each of the pair of opposing nozzles variable; a slit width adjusting mechanism for adjusting the edge positions of the slit to the edge positions of the steel strip; and a gas flow rate adjusting mechanism for achieving a uniform velocity of the flow discharged out of the nozzle.

This gas wiping device adjusts the edge positions of the slit of each of the pair of nozzles opposed to each other across the steel strip to the edge positions of the steel strip, so as to obtain a state in which the jet flows from the opposing nozzles do not strongly collide with each other, thereby eliminating the turbulence caused by the collision of the jet flows. In this way, the distribution of the molten metal that becomes attached onto the steel strip surface is made uniform as much as possible, whereby the splashing and the overcoating at the edges are described to be suppressed.

However, in the gas wiping device disclosed in Patent Document 3, only the gas outlet is blocked to decrease the gas spraying width. Thus, the gas that has been circulated through the hollow of the nozzle is considerably contracted by the outlet. The contracted flow periodically produces vortexes, which disturb the gas flow and cause intermittent overcoating or splashing at the edges of the steel strip in the width direction. Accordingly, the overcoating or splashing cannot be completely suppressed.

The above will be described with reference to a schematic diagram shown in FIG. 11, schematically illustrating a gas wiping device W according to Patent Document 1. Two blocking members H, H are slidably (Y1-direction) disposed in a front portion, and the width of a central gas outlet E enclosed by the blocking members H, H is variably adjusted as the blocking members H, H are slid. A gas introduced from the rear of the gas wiping device W (X3-direction) flows forward via the hollow of the gas wiping device W, and is discharged via the gas outlet E (X4-direction). The flow of the gas that has reached the blocking members H, H via the hollow is sharply contracted toward the center (X5-direction), whereby the above-described vortexes are produced. The vortexes disturb the flow of gas, thereby causing intermittent overcoating or splashing at the edges of the steel strip in the width direction.

### PRIOR ART DOCUMENT

Patent Document 1: JP Patent Publication (Yoshihiro) JP 2006-274381 A1
Patent Document 2: US Patent Publication (Bottaro) US 3,977,359 A
Patent Document 3: JP Patent Publication (Kokai) No. 2007-284732 A1

### SUMMARY OF THE INVENTION

### PROBLEM TO BE SOLVED BY THE INVENTION

The present invention was made in view of the above problem, and relates to a gas wiping device including a gas wiping nozzle for adjusting the amount of molten metal for plating attached to a surface of a steel strip by spraying gas onto the surface. An object of the present invention is to provide a gas wiping device that can highly effectively suppress overcoating or splashing at the edges of the steel strip in the width direction.

### MEANS FOR SOLVING THE PROBLEM

In order to achieve the object, a gas wiping device according to the present invention includes a hollow gas wiping nozzle for adjusting the amount of molten metal for plating attached to a surface of a steel strip by spraying a gas onto the surface. The gas wiping nozzle includes a slit extending along a width direction of the steel strip for blowing the gas out of the hollow, and a partition wall having a gas introducing opening for introducing the gas into the hollow. The slit is provided with left and right blocking members for blocking left and right areas in accordance with a width of the steel strip, the left and right blocking members being slidable along the slit, with a gas outlet formed between the left and right blocking members spaced apart from each other. In the hollow, left and right rectification pieces extending from respective gas outlet side ends of the left and right blocking members toward the partition wall are disposed, with a gas flow passageway formed between the left and right rectification pieces. The gas outlet and the gas flow passageway have the same width, and the left and right rectification pieces extend from the top surface to the bottom surface of the hollow.

The gas wiping nozzle of the gas wiping device according to the present invention is opposed to the steel strip, and the elongated slit extending along the width direction of the steel strip is provided with the left and right blocking members that block the left and right areas of the slit and that are slidable along the slit. The gas outlet is formed between the left and right blocking members of the slit, and the width of the gas outlet can be freely adjusted by sliding the left and right blocking members. The mode of sliding of the left and right blocking members includes a mode such that the left and right blocking members are slid in a synchronized manner and by the same amount, and a mode such that only one of the left and right blocking members is slid. By sliding the left and right blocking members, the width of the gas outlet can be adjusted to be approximately the same as the width of the steel strip. More specifically, the width of the steel strip on the order of 700 mm to 1800 mm may be adjusted to be the same as the width of the gas outlet, or the width of the gas outlet may be adjusted to extend beyond each of the left and right edges of the steel strip by approximately 10 mm.

In the hollow of the gas wiping nozzle, the left and right rectification pieces extending from the left and right edges of the gas introducing opening to the respective gas outlet side ends of the left and right blocking members are disposed, the left and right rectification pieces defining the gas flow passageway in the hollow. Thus, of the gas introduced via the gas introducing opening, particularly the gas that flows along the rectification pieces at the left and right ends of the gas flow passageway can be smoothly discharged out of the gas outlet via the rectification pieces and the continuous gas outlet side ends of the blocking members.

Namely, the considerable (sharp) contraction, by the gas outlet, of the gas that has been circulated through the hollow of the gas wiping nozzle, and the resultant generation of the periodic vortexes that disturb the flow of gas, do not occur. Thus, the overcoating or splashing at the width direction edges of the steel strip due to the flow of gas disturbed by the generated vortexes can be completely eliminated.

In the present specification, regarding the terms "left and right", the width direction of the steel strip as it is transported upward from the plating pot is defined as a left/right direction. Thus, references to the "left and right" of the steel strip, the "left and right" areas of the slit, and the "left and right" edges of the gas introducing opening are with respect to the width direction of the steel strip.

The width of the gas flow passageway defined by the left and right rectification pieces in the hollow of the gas wiping nozzle, and the width of the gas outlet are constantly maintained to be the same. When the width of the gas outlet is varied by the sliding of the left and right blocking members, the variation is tracked by sliding the left and right rectification pieces so that the width of the gas flow passageway and the width of the gas outlet are varied in the same state. Because the left and right rectification pieces are slid, the rectification pieces according to the present embodiment are structurally separated from the partition wall.

In a preferred embodiment of the gas wiping device according to the present invention, the gas wiping nozzle may include a hanging piece fixed to an upper surface of the hollow, the hanging piece not reaching a lower surface, and a rising piece fixed to the lower surface at a position spaced apart from the hanging piece, the rising piece not reaching the upper surface, and the gas introduced into the gas flow passageway via the gas introducing opening may be rectified in a process of being circulated along the hanging piece and the rising piece.

Because the hanging piece and the rising piece are disposed at an interval in the gas flow passageway, the gas is rectified as it is circulated along the hanging piece and the rising piece in a meandering manner, whereby the gas pressure or flow velocity in the width direction of the gas flow passageway is made as uniform as possible.

In an embodiment related to the sliding control of the left and right blocking members, the left and right blocking members may be configured to be slidable by a left sliding mechanism and a right sliding mechanism, respectively, as specific sliding mechanisms; the left sliding mechanism and the right sliding mechanism may be mounted on a common base, the base being connected to a base sliding mechanism and slidable; a position sensor for detecting a steel strip position may be disposed near the gas outlet; the left sliding mechanism and the right sliding mechanism may be configured to slide the left and right blocking members to adjust the width of the gas outlet; and the base sliding mechanism may be configured to slide the base based on steel strip position data detected by the position sensor, the sliding of the base causing the right sliding mechanism and the left sliding mechanism to slide, thus causing the left and right blocking members to slide while the already adjusted width of the gas outlet is maintained.

According to the present embodiment, the sliding control of the left and right blocking members is implemented by the specific sliding mechanisms, i.e., the left sliding mechanism and the right sliding mechanism, respectively. The sliding mechanism may include a cylinder device for sliding the blocking member, or an electric slider device that slides over a slide substrate. When the cylinder device is used, the device may include a slidable piston with the blocking member attached to the end of the piston, so that the blocking member can be slid to the left or right as the piston is slidably moved. When the electric slider device is used, an electric slider and the blocking member may be connected via a wire and the like, so that the blocking member can be slid to the left or right in accordance with the sliding of the electric slider to the left or right on the slide substrate.

For example, data about the width of the steel strip inputted to a process computer is transmitted to the left and right sliding mechanisms, and the left and right sliding mechanisms are slid based on the transmitted data, thus adjusting the width of the gas outlet to a desired width.

The steel strip transported from the reduction annealing furnace is immersed in the molten metal in the plating pot, and then vertically upwardly transported via the sink roll in the plating pot. Some of the molten metal that becomes attached to both sides of the steel strip is removed by the gas blown out of the gas wiping devices disposed on both sides of the transport path of the vertically upward transported steel strip, whereby the attached molten metal is adjusted to a desired attached amount. Although the width of the gas outlet is adjusted to the desired width based on the data about the width of the steel strip, the steel strip may meander during the transport process. As a result, the center line of the steel strip may often be displaced from the center line of the gas outlet with an already adjusted width.

Thus, according to the present embodiment, the left sliding mechanism and the right sliding mechanism are mounted on the common base, and the base is connected to the base sliding mechanism and configured to be slidable. Further, the position sensor for detecting the steel strip position is disposed near the gas outlet, and the base sliding mechanism slides the base as desired based on steel strip position data from the position sensor (center line position data of the steel strip, or position data of the left and right edges of the steel strip), whereby the left and right sliding mechanisms are slid to correspond to the steel strip position without changing the relative positions of the left and right sliding mechanisms defining the width of the gas outlet.

The base sliding mechanism may include a cylinder device or an electric slider device, as in the case of the left and right sliding mechanisms. Regarding the position sensor for detecting the steel strip position disposed near the gas outlet, while it may be preferable to dispose the position sensor as near to the gas outlet as possible from the viewpoint of blowing the gas against the steel strip more accurately, the term "near" herein may include a relatively wide range, extending from the bath level in the pot to an area above the gas wiping device, for example.

In another embodiment related to the sliding control of the left and right blocking members, the left and right blocking members may be configured to be slidable by a left sliding mechanism and a right sliding mechanism, respectively, as specific sliding mechanisms; a position sensor for detecting a steel strip position may be disposed near the gas outlet; the left sliding mechanism and the right sliding mechanism may be configured to slide the left and right blocking members so as to adjust the width of the gas outlet; and the left sliding mechanism and the right sliding mechanism may be configured to slide the left and right blocking members based on steel strip position data detected by the position sensor, while the already adjusted width of the gas outlet is maintained.

According to the present embodiment, while the width of the gas outlet is adjusted by the left sliding mechanism and the right sliding mechanism, as according to the foregoing embodiments, the left and right sliding mechanisms are not mounted on a common base. The left and right sliding mechanisms are slid in a synchronized manner in the same direction and by the same amount based on the steel strip position information data received from the position sensor, whereby the left and right blocking members are controlled to be slid to correspond to the steel strip position while the already adjusted width of the gas outlet is maintained.

Preferably, the left and right edges of the steel strip and the respective gas outlet side ends of the left and right blocking members may have gaps of the same adjusted length s, where s is in a range of 0 ≤ s ≤ 10 mm.

Based on the results of investigations by the present inventors, it has been proved that there is no or very little splashing and that no clogging of the nozzle is caused when the gap s between the left and right edges of the steel strip and the respective gas outlet side ends of the left and right blocking members is in the rage of 0 ≤ s ≤ 10 mm.

### EFFECTS OF THE INVENTION

As will be understood from the above, the gas wiping device according to the present invention is provided with the extremely simple structural improvement that the gas outlet side ends of the left and right blocking members in the slit forming the gas outlet are connected to the left and right rectification pieces defining the gas flow passageway in the hollow of the gas wiping nozzle. As a result, the generation of periodic vortexes by considerable flow contraction of the gas circulated through the hollow of the gas wiping nozzle by the gas outlet, and the resultant disturbance of the flow of gas by the vortexes, are eliminated. Thus, the overcoating or splashing at the width direction edges of the steel strip due to the disturbed flow of gas can be completely eliminated.

### BRIEF DESCRIPTION OF THE DRAWINGS

FIG. 1 is a schematic diagram illustrating a configuration of a molten metal plating apparatus.
FIG. 2 is a perspective view of an embodiment of a gas wiping device.
FIG. 3 is a III-III sagittal view of FIG. 2.
FIG. 4 is a IV-IV sagittal view of FIG. 3.
FIG. 5 is a cross sectional view of another embodiment of the gas wiping device, corresponding to FIG. 3.
FIG. 6 is a VI-VI sagittal view of FIG. 5.
FIG. 7 is a schematic diagram of an embodiment of a sliding mechanism for left and right blocking members.
FIG. 8 is a schematic diagram of another embodiment of the sliding mechanism for the left and right blocking members.
FIG. 9(a) is a longitudinal cross sectional view of an analysis model, and FIG. 9(b) is a b-b sagittal view of FIG. 9(a).
FIG. 10(a) illustrates an analysis result for a comparative example, and FIG. 10(b) illustrates an analysis result for an example.
FIG. 11 is a schematic diagram illustrating a sharp contraction of gas caused by slidable blocking members in a conventional gas wiping device.

### MODE FOR CARRYING OUT THE INVENTION

In the following, embodiments of the gas wiping device according to the present invention will be described with reference to the drawings.

### (Plating apparatus)

FIG. 1 is a schematic diagram of a molten metal plating apparatus. The plating apparatus includes a plating pot Y containing plating bath of a molten metal M of molten zinc or molten aluminum, with the inside of the plating pot Y lined with fire bricks and the like, which are not illustrated. In the plating pot Y, a sink roll R is rotatably disposed. A steel strip K transferred from a reduction annealing furnace via a snout and the like, which are not illustrated, is immersed in the molten metal M and then transported vertically upward via the sink roll R (X1-direction).

The steel strip K transported vertically upward has molten metal attached onto both sides thereof. Above the plating pot Y, gas wiping devices 10, 10 are disposed on both sides of the vertically upward transport path of the steel strip K. The gas wiping devices 10, 10 blow out a gas (air, nitrogen, inert gas, or the like) in order to remove a part of the molten metal that is attached onto the both sides of the steel strip K, thus adjusting the attached molten metal to a desired amount.

### (First embodiment of gas wiping device)

FIG. 2 is a perspective view of an embodiment of the gas wiping devices of the plating apparatus of FIG. 1. FIG. 3 is a III-III sagittal view of FIG. 2. FIG. 4 is a IV-IV sagittal view of FIG. 3.

The gas wiping device 10 illustrated in FIGS. 2 to 4 includes a hollow gas wiping nozzle 1, and a gas supply device (gas supply source), not illustrated, which is disposed behind the gas wiping nozzle 1 and configured to supply the gas to gas inlet pipes 1b via which the gas is supplied into the hollow of the gas wiping nozzle 1.

The gas wiping nozzle 1 includes a slit 1a' (with a full width T) extending in a width direction of the steel strip K for blowing the gas out of the hollow. In the slit 1a', left and right blocking members 2, 2 for blocking left and right areas of the slit 1a' are disposed slidably along the slit 1a' (direction Y1). A gas outlet 1a is formed between a slit area between the left and right blocking members 2, 2 spaced apart from each other.

The gas inlet pipes 1b are in communication with the inside of the gas wiping nozzle 1 at a rear portion thereof, and a partition wall 1d with a plurality of gas introducing openings 1e is disposed at the front of the rear portion. The gas supplied via the gas supply device, not illustrated, is introduced into the gas wiping nozzle 1 via the gas inlet pipes 1b (X2-direction), and is further introduced into the hollow via the gas introducing openings 1e.

In the hollow of the gas wiping nozzle 1, left and right rectification pieces 1c, 1c are disposed, extending from respective gas outlet side ends 2a, 2a of the left and right blocking members 2, 2 toward the partition wall 1d. A space defined by the left and right rectification pieces 1c, 1c and the upper and lower surfaces of the hollow provides a gas flow passageway GR.

The gas wiping device 10 is configured such that the gas flow passageway GR formed between the left and right rectification pieces 1c, 1c has a width t which is the same as a width t of the gas outlet 1a at all times. Namely, the left and right rectification pieces 1c, 1c are orthogonally fixed at one ends to the gas outlet side ends 2a, 2a of the left and right blocking members 2, 2, respectively, with the other ends of the left and right rectification pieces 1c, 1c completely separated from the partition wall 1d. Thus, the width t of the gas outlet 1a and the width t of the gas flow passageway GR can be variably adjusted by the same width.

By sliding the left and right blocking members 2, 2 (Y1-direction), the width t of the gas outlet 1a can be freely adjusted. For example, in an adjustment mode, the width t of the gas outlet 1a is adjusted to be the same as the width of the steel strip K, which may vary between approximately 700 mm to 1800 mm. In another adjustment mode, the width t of the gas outlet 1a may be adjusted to extend beyond each of the left and right edges of the steel strip K by approximately 10 mm. Thus, the width t of the gas outlet 1a can be adjusted as desired in accordance with a variation in the width of the steel strip K.

The sliding mode of the left and right blocking members 2, 2 includes a mode in which both are slid by the same amount in a synchronized manner, and a mode in which only one of the left and right blocking members is slid.

As will be seen from FIG. 3, of the gas introduced into the gas flow passageway GR via the gas introducing openings 1e (X3-direction), particularly the gas that flows along the rectification pieces 1c, 1c at the left and right ends of the gas flow passageway GR is smoothly discharged out of the gas outlet 1a via the rectification pieces 1c, 1c and the continuous gas outlet side ends 2a of the blocking members 2 (X4-direction).

Namely, the sharp contraction, by the gas outlet 1a, of the gas that has been circulated through the hollow of the gas wiping nozzle 1, and the resultant periodic generation of the vortexes that disturb the flow of gas, do not occur. Thus, the overcoating or splashing at the edges of the steel strip in the width direction due to the flow of gas disturbed by the produced vortexes can be completely eliminated.

### (Second embodiment of gas wiping device)

FIG. 5 is a cross sectional view of another embodiment of the gas wiping device, illustrated in a manner corresponding to FIG. 3. FIG. 6 is a VI-VI sagittal view of FIG. 5.

The illustrated gas wiping device 10A includes a hanging piece 3a fixed to an upper surface of the hollow in the gas flow passageway GR, the hanging piece 3a not reaching a lower surface. At a position spaced apart from the hanging piece 3a on the lower surface of the hollow, a rising piece 3b that does not reach the upper surface is fixed. Thus, the gas introduced into the gas flow passageway GR via the gas introducing openings 1e is rectified in the process (X3') of being circulated along the hanging piece 3a and the rising piece 3b.

The other ends of the left and right rectification pieces 1c, 1c are located forwardly of the rising piece 3b and the hanging piece 3a, so that the left and right rectification pieces 1c, 1c can be slid in front of the rising piece 3b and the hanging piece 3 a as the width of the gas outlet 1a is varied.

By such rectification, the flow velocity or pressure of the gas introduced via the gas introducing openings 1e is made as uniform as possible with respect to the width direction of the gas flow passageway GR, whereby the gas having a uniform flow velocity or pressure can be provided along the width direction of the steel strip K.

In the gas wiping device 10A according to the present embodiment, too, of the gas introduced into the gas flow passageway GR via the gas introducing openings 1e, particularly the gas that flows along the rectification pieces 1c, 1c at the left and right ends of the gas flow passageway GR is smoothly discharged out of the gas outlet 1a via the rectification pieces 1c and the continuous gas outlet side ends 2a of the blocking members 2, so that the generation of the vortexes and the resultant disturbance of the flow of gas do not occur.

### (First embodiment of sliding mechanism for left and right blocking members)

With reference to FIG. 7, a first embodiment of a sliding mechanism for the left and right blocking members of the gas wiping device 10 will be described.

In the illustrated sliding mechanism, the left and right blocking members 2, 2 are slidable to the left and right by their specific left sliding mechanism 5A and right sliding mechanism 5B. The left sliding mechanism 5A and the right sliding mechanism 5B are mounted on a common base 6. The common base 6 is connected to a base sliding mechanism 7 and configured to be slidable.

The left blocking member 2 and an electric slider constituting the left sliding mechanism 5A are connected substantially in a ring shape by two wires W1, W1 via pulleys 9. Thus, when the left sliding mechanism 5A is slid to the left or right (Z1-direction), the left blocking member 2 is can also be slid to the left or right in a synchronized manner (Z1'-direction). Similarly, the right blocking member 2 and an electric slider constituting the right sliding mechanism 5B are connected by two wires W2, W2 in a substantially ring shape via pulleys 9. Thus, when the right sliding mechanism 5B is slid to the left or right (Z2-direction), the right blocking member 2 is also slid to the left or right in a synchronized manner (Z2'-direction).

Further, the common base 6 on which the left sliding mechanism 5A and the right sliding mechanism 5B are mounted is slidable by an electric cylinder constituting the base sliding mechanism 7. With the left and right sliding mechanisms 5A and 5B, which enable the sliding of the left and right blocking members 2, 2 positioned to define the gas outlet 1a of the desired width t, fixedly positioned, the base sliding mechanism 7 is controlled to slide the base 6, whereby a center line CL2 of the steel strip K as it meanders during transport and a center line CL1 of the gas outlet 1a are aligned.

Specifically, data concerning the width of the steel strip K being transported is transmitted from a process computer PC to the left and right sliding mechanisms 5A and 5B, and the left and right sliding mechanisms 5A and 5B are slid based on the transmitted signal, whereby the left and right blocking members 2, 2 are slid to form the gas outlet 1a with a desired width t.

Meanwhile, two sets of position sensors 4, 4 are disposed near the gas outlet 1a to sense the steel strip K in the vicinity of the left and right edges thereof as the steel strip K travels along the transport path, and obtained sensing data is transmitted to the base sliding mechanism 7. Based on the sensing data from the left and right position sensors 4, 4, the center line CL2 of the steel strip K near the gas outlet 1a is determined. When the center line CL2 is not aligned with the center line CL1 of the gas outlet 1a, the base sliding mechanism 7 and the base 6 are slid (Z3-direction) by an amount corresponding to the difference. As the base 6 is slid, the left and right sliding mechanisms 5A and 5B mounted thereon are slid in a synchronized manner, and the left and right blocking members 2, 2 are slid correspondingly to align the center lines CL1 and CL2 of the gas outlet 1a and the steel strip K.

### (Second embodiment of sliding mechanism for left and right blocking members)

With reference to FIG. 8, a second embodiment of the sliding mechanism for the left and right blocking members of the gas wiping device 10 will be described.

The sliding mechanism illustrated in FIG. 8 differs from the sliding mechanism of FIG. 7 in that the left and right sliding mechanisms 5A and 5B are not mounted on a common base; that the left and right sliding mechanisms 5A and 5B, after the gas outlet 1a with the desired width t is formed, are slid in a synchronized manner and by the same amount in accordance with the meandering of the steel strip K, thus tracking the steel strip K as it meanders; and that only the right edge ed of the steel strip K is sensed by a single position sensor 4A which is slidable by a position sensor sliding mechanism 8.

The right edge ed of the steel strip K is sensed while the position sensor 4A is slid by the position sensor sliding mechanism 8 to track the steel strip K as it meanders, and the sensing data is transmitted to the left and right sliding mechanisms 5A and 5B. The left and right sliding mechanisms 5A and 5B are slid in the same direction and by the same amount, whereby the left and right blocking members 2, 2 are slid in the same direction and by the same amount. Thus, the right edge ed of the steel strip K is controlled to be positioned at a desired position with respect to the gas outlet 1a.

### [Turbulence analysis investigating the degree of splashing, and its result]

The present inventors created an analysis model simulated as illustrated in FIG. 9(a) and (b) using a computer, and performed an LES turbulence analysis (LES: a non-steady turbulence analysis method by which a vortex greater than an analysis cell is directly calculated rather than modeled). As illustrated in FIG. 9(b), a steel strip had a width t1 of 150 mm; an inner width t2 of the gas discharge opening and a gas spraying width t3 were both 150 mm; the gas discharge opening had a height t4 of 1.2 mm; and the two gas wiping devices opposed to each other across the steel strip had a gas discharge opening interval t5 of 20 mm. An internal air pressure in the gas discharge opening was 40 kPa.

The modeling involved modeling a half area with respect to the center of the steel strip, as illustrated in FIG. 9(b) (the total number of cells of the model was 2,654,640). Of an analysis result chart formed on a computer screen, an analysis result chart modeling the conventional example of FIG. 11 is illustrated in FIG. 10(a), while an analysis result chart modeling an example according to the present invention is illustrated in FIG. 10(b).

In a right edge area of FIG. 10(a), the air flow directions are inclined in diagonally upper-right and lower-right directions (which proves that the splashes are large). In a right portion area of FIG. 10(b), the air flow directions are inclined in the upper-right or lower-right direction in significantly smaller proportions, thus proving that the occurrence of splashing is extremely small.

### [Experiment regarding range of steel strip feeding rate (transport rate) during plating process, and its result]

The present inventors conducted an experiment to identify a possible range concerning steel strip feeding rate in the case of the gas wiping device illustrated in FIGS. 3 and 4 (example) and the case of the conventional gas wiping device illustrated in FIG. 11 (comparative example). Specifically, when the steel strip had a thickness of 0.4 mm and a width of 1200 mm, and the gap between the left and right edges of the steel strip and the edges of the gas outlet was 0 mm, a strip feeding rate range such that the amount of zinc as a plating molten metal that became attached to both sides of the steel strip was 120 g/m² was investigated. The present experiment was not conducted with regard to the gas wiping device according to the second embodiment illustrated in FIGS. 5 and 6. However, it should be noted that obviously the gas wiping device according to the second embodiment would provide an even higher effect than the effect of the experiment on the gas wiping device according to the first embodiment illustrated in FIGS. 3 and 4 because a further gas rectification effect can be expected from the hanging piece and the rising piece.

Table 1 shows the result of the experiment. In Table 1, "Good" indicates that there was little splashing and no re-attachment onto the steel strip; "Poor" indicates that, while there was some attachment to the nozzle due to splashing, there was no re-attachment to the steel strip; and "Bad" indicates there was much splashing, causing attachment to the nozzle and re-attachment to the steel strip.

As shown in Table 1, in the case of the gas wiping device according to the example, it was confirmed that there was no re-attachment of splashing onto the steel strip when the strip feeding was conducted in a strip feeding rate range of up to 240 mpm.

On the other hand, the strip feeding rate range such that a similar effect could be expected from the gas wiping device according to the comparative example was a range of up to 180 mpm.

Thus, the experimental result proves that, compared with the use of the conventional gas wiping device, an operation with a 30% or more increase in strip feeding rate can be performed.

**Table 1**

| | | Comparative example (model of FIG. 11) | | | | Example (FIG. 1) | | | |
|---|---|---|---|---|---|---|---|---|---|
| N₂ gas source pressure (kPa) | Strip feeding rate (mpm) | Gap | | | | Gap | | | |
| | | 0 mm | 5 mm | 10 mm | 15 mm | 0 mm | 5 mm | 10 mm | 15 mm |
| 40 | 160 | Good | Good | Good | Poor | Good | Good | Good | Poor |
| 50 | 180 | Poor | Poor | Poor | Bad | Good | Good | Good | Poor |
| 70 | 200 | Bad | Bad | Bad | Bad | Good | Good | Good | Poor |
| 90 | 220 | Bad | Bad | Bad | Bad | Good | Good | Good | Bad |
| 110 | 240 | Bad | Bad | Bad | Bad | Poor | Poor | Poor | Bad |
| 130 | 250 | Bad | Bad | Bad | Bad | Bad | Bad | Bad | Bad |

### [Experiment investigating an optimum range of gap between left and right edges of steel strip and gas outlet edges, and its result]

The present inventors further conducted an experiment regarding the magnitude of the problem of splashing and the presence or absence of re-attachment to the steel strip with varying gaps between the left and right edges of the steel strip and the gas outlet edges. The various conditions and the experimental result are shown in Table 1.

The experimental result indicates that the example provides good results even in higher gas source pressure and strip feeding rate ranges compared with the comparative example. The experimental result for the example also proves that the gap between the left and right edges of the steel strip and the gas outlet edges is preferably in a range of from 0 mm to 10 mm.

While the embodiments of the present invention have been described with reference to the drawings, specific configurations are not limited to the embodiments, and design variations and the like within the scope of the present invention shall be included in the present invention.

### REFERENCE SIGNS LIST

- 1: Gas wiping nozzle
- 1a: Gas outlet
- 1a': Slit
- 1b: Gas inlet pipe
- 1c: Rectification piece
- 1d: Partition wall
- 1e: Gas introducing opening
- 2: Blocking member
- 2a: Gas outlet side edge of blocking member
- 3a: Hanging piece
- 3b: Rising piece
- 4, 4A: Position sensor
- 5A: Left sliding mechanism
- 5B: Right sliding mechanism
- 6: Base (common base)
- 7: Base sliding mechanism
- 8: Position sensor sliding mechanism
- 10, 10A: Gas wiping device
- M: Molten metal (plating bath)
- K: Steel strip
- Y: Plating pot
- R: Sink roll
- W1, W2: Wire
- PC: Process computer
- CL1: Center line of gas outlet
- CL2: Center line of steel strip
- ed: Right edge of steel strip

## Claims

1. A gas wiping device (10) comprising a hollow gas wiping nozzle (1) for adjusting the amount of molten metal for plating attached to a surface of a steel strip (K) by spraying a gas onto the surface,
wherein:
the gas wiping nozzle (1) includes a slit (1a') extending along a width direction of the steel strip for blowing the gas out of the hollow, and a partition wall (1d) having a gas introducing opening (1e) for introducing the gas into the hollow;
the slit (1a') is provided with left and right blocking members (2, 2) for blocking left and right areas in accordance with a width of the steel strip, the left and right blocking members being slidable along the slit (1a'), with a gas outlet (1a) formed between the left and right blocking members (2, 2) spaced apart from each other;
in the hollow, left and right rectification pieces (1c, 1c) extending from respective gas outlet side ends (2a, 2a) of the left and right blocking members (2,2) toward the partition wall (1d) are disposed, with a gas flow passageway (GR) formed between the left and right rectification pieces (1c, 1c);
the gas outlet (1a) J and the gas flow passageway (GR) J have the same width; and
the left and right rectification pieces (1c, 1c) extend from the top surface to the bottom surface of the hollow.

2. The gas wiping device according to claim 1, wherein the left and right blocking members (2, 2) and the left and right rectification pieces (1c, 1c) are configured to be slid in a synchronized manner so as to adjust the width of the gas outlet (1a) and the width of the gas flow passageway (GR).

3. The gas wiping device according to claim 1 or 2, wherein:
the gas wiping nozzle (1) includes a hanging piece (3a) fixed to an upper surface of the hollow, the hanging piece (3a) not reaching a lower surface, and a rising piece (3b) fixed to the lower surface at a position spaced apart from the hanging piece (3a), the rising piece (3b) not reaching the upper surface; and
the gas introduced into the gas flow passageway via the gas introducing opening (1e) is rectified in a process of being circulated along the hanging piece (3a) and the rising piece (3b)

4. The gas wiping device according to any one of claims 1 to 3, wherein:
the left and right blocking members (2, 2) are slidable by a left sliding mechanism (5A) and a right sliding mechanism (5B), respectively, as specific sliding mechanisms;
the left sliding mechanism (5A) and the right sliding mechanism (5B) are mounted on a common base (6), the base being connected to a base sliding mechanism (7) and slidable;
a position sensor (4) for detecting a steel strip position is disposed near the gas outlet (1a);
the left sliding mechanism (5A) and the right sliding mechanism (5B) are configured to slide the left and right blocking members (2, 2) to adjust the width of the gas outlet; and
the base sliding mechanism (7) is configured to slide the base based on steel strip position data detected by the position sensor (4),
the sliding of the base causing the right sliding mechanism (5B) and the left sliding mechanism (5A) to slide, thus causing the left and right blocking members (2,2) to slide while the already adjusted width of the gas outlet is maintained.

5. The gas wiping device according to any one of claims 1 to 3, wherein:
the left and right blocking members (2, 2) are slidable by a left sliding mechanism (5A) and a right sliding mechanism (5B), respectively, as specific sliding mechanisms;
a position sensor (4) for detecting a steel strip position is disposed near the gas outlet (1a);
the left sliding mechanism (5A) and the right sliding mechanism (5B) are configured to slide the left and right blocking members (2, 2) so as to adjust the width of the gas outlet; and
the left sliding mechanism (5A) and the right sliding mechanism (5B) are configured to slide the left and right blocking members (2, 2) based on steel strip position data detected by the position sensor while the already adjusted width of the gas outlet is maintained.

## Patentansprüche

1. Gasabstreifvorrichtung (10), umfassend eine hohle Gasabstreifdüse (1) zur Einstellung der Menge an geschmolzenem Metall zur Plattierung einer Oberfläche eines Stahlstreifens (K) durch Sprühen von Gas auf die Oberfläche, wobei:
die Gasabstreifdüse (1) einen Schlitz (1a') umfasst, der sich entlang einer Breitenrichtung des Stahlstreifens erstreckt, zum Ausblasen von Gas aus dem Hohlraum, und eine Trennwand (1d) mit einer Gaseinleitungsöffnung (1e) zur Einleitung von Gas in den Hohlraum;
wobei der Schlitz (1a') mit linken und rechten Blockierungselementen (2, 2) zur Blockierung linker und rechter Bereiche in Übereinstimmung mit einer Breite des Stahlstreifens versehen ist, wobei die linken und rechten Blockierungselemente entlang des Schlitzes (1a') verschiebbar sind, wobei ein Gasauslass (1a) zwischen den linken und rechten Blockierungselementen (2, 2), die voneinander beabstandet sind, ausgebildet ist;
wobei in dem Hohlraum linke und rechte Ausrichtstücke (1c, 1c) angeordnet sind, die sich von jeweiligen Gasauslass-Seitenenden (2a, 2a) der linken und rechten Blockierungselemente (2, 2) zu der Trennwand (1d) hin erstrecken, wobei ein Gasströmungsdurchgang (GR) zwischen den linken und rechten Ausrichtstücken (1c, 1c) ausgebildet ist;
wobei der Gasauslass (1a) und der Gasströmungsdurchgang (GR) dieselbe Breite aufweisen; und
die linken und rechten Ausrichtstücke (1c, 1c) sich von der oberen Oberfläche zu der unteren Oberfläche des Hohlraums erstrecken.

2. Gasabstreifvorrichtung nach Anspruch 1, wobei die linken und rechten Blockierungselemente (2, 2) und die linken und rechten Ausrichtstücke (1c, 1c) dazu ausgestaltet sind, auf synchronisierte Weise verschoben zu werden, um so die Breite des Gasauslasses (1a) und die Breite des Gasströmungsdurchgangs (GR) einzustellen.

3. Gasabstreifvorrichtung nach Anspruch 1 oder 2, wobei:
die Gasabstreifdüse (1) ein hängendes Stück (3a) umfasst, das an einer oberen Oberfläche des Hohlraums fixiert ist, wobei das hängende Stück (3a) eine untere Oberfläche nicht erreicht, und ein hochragendes Stück (3b), das an der unteren Oberfläche an einer Position, die von dem hängenden Stück (3a) beabstandet ist, angeordnet ist, wobei das hochragende Stück (3b) die obere Oberfläche nicht erreicht; und
das in den Gasströmungsdurchgang über die Gaseinleitungsöffnung (1e) eingeleitete Gas in einem Verfahren ausgerichtet wird, in dem es entlang des hängenden Stücks (3a) und des hochragenden Stücks (3b) zirkuliert wird.

4. Gasabstreifvorrichtung nach einem der Ansprüche 1 bis 3, wobei:
die linken und rechten Blockierungselemente (2, 2) durch einen linken Verschiebemechanismus (5A) und einen rechten Verschiebemechanismus (5B) als jeweils eigenständige Verschiebemechanismen verschiebbar sind;
wobei der linke Verschiebemechanismus (5A) und der rechte Verschiebemechanismus (5B) an einer gemeinsamen Basis (6) montiert sind, wobei die Basis mit einem Basis-Verschiebemechanismus (7) verbunden und verschiebbar ist;
wobei ein Stellungssensor (4) zur Erfassung der Stellung eines Stahlstreifens nahe an dem Gasauslass (1a) angeordnet ist;
wobei der linke Verschiebemechanismus (5A) und der rechte Verschiebemechanismus (5B) dazu ausgestaltet sind, die linken und rechten Blockierungselemente (2, 2) zu verschieben, um die Breite des Gasauslasses einzustellen; und
wobei der Basis-Verschiebemechanismus (7) dazu ausgestaltet ist, die Basis auf der Grundlage von Stahlstreifen-Stellungsdaten zu verschieben, die durch den Stellungssensor (4) erfasst werden, wobei das Verschieben der Basis die Verschiebung des rechten Verschiebemechanismus (5B) und des linken Verschiebemechanismus (5A) verursacht, und somit die Verschiebung der linken und rechten Blockierungselemente (2, 2) verursacht, während die bereits eingestellte Breite des Gasauslasses beibehalten wird.

5. Gasabstreifvorrichtung nach einem der Ansprüche 1 bis 3, wobei:
die linken und rechten Blockierungselemente (2, 2) durch einen linken Verschiebemechanismus (5A) und einen rechten Verschiebemechanismus (5B) als jeweils eigenständige Verschiebemechanismen verschiebbar sind;
wobei ein Stellungssensor (4) zur Erfassung der Stellung eines Stahlstreifens nahe an dem Gasauslass (1a) angeordnet ist;
wobei der linke Verschiebemechanismus (5A) und der rechte Verschiebemechanismus (5B) dazu ausgestaltet sind, die linken und rechten Blockierungselemente (2, 2) zu verschieben, um so die Breite des Gasauslasses einzustellen; und
wobei der linke Verschiebemechanismus (5A) und der rechte Verschiebemechanismus (5B) dazu ausgestaltet sind, die linken und rechten Blockierungselemente (2, 2) auf der Grundlage von Stahlstreifen-Stellungsdaten zu verschieben, die durch den Stellungssensor erfasst werden, während die bereits eingestellte Breite des Gasauslasses beibehalten wird.

## Revendications

1. Dispositif de raclage par gaz (10), comportant une buse creuse de raclage par gaz (1) pour ajuster la quantité du métal fondu pour plaquer la surface d'une bande d'acier (K) en atomisant un gaz sur la surface, dans lequel :
la buse de raclage par gaz (1) comprend une fente (1a') s'étendant le long d'une direction de largeur de la bande d'acier pour souffler le gaz à partir de la cavité, et une cloison (1d) avec une ouverture d'introduction de gaz (1e) pour introduire le gaz dans la cavité ;
la fente (1a') est prévue des éléments de blocage gauches et droits (2, 2) pour bloquer des régions gauches et droites en accord avec la largeur de la bande d'acier, les éléments de blocage gauches et droits pouvant coulisser le long de la fente (1a'), avec une sortie de gaz (1a) formée entre les éléments de blocage gauches et droits (2, 2) espacés l'un de l'autre ;
dans la cavité sont disposés des organes rectificateurs gauches et droits (1c, 1c) s'étendant à partir des extrémités latérales de sortie de gaz (2a, 2a) respectives des éléments de blocage gauches et droits (2, 2) vers la cloison (1d), avec un passage d'écoulement de gaz (GR) formé entre les organes rectificateurs gauches et droits (1c, 1c) ;
la sortie de gaz (1a) et le passage d'écoulement de gaz (GR) ont la même largeur ; et
les organes rectificateurs gauches et droits (1c, 1c) s'étendent à partir d'une surface supérieure vers une surface inférieure de la cavité.

2. Dispositif de raclage par gaz selon la revendication 1, dans lequel les éléments de blocage gauches et droits (2, 2) et les organes rectificateurs gauches et droits (1c, 1c) sont configurés pour être déplacés de manière synchronisée pour ajuster la largeur de la sortie de gaz (1a) et la largeur du passage d'écoulement de gaz (GR).

3. Dispositif de raclage par gaz selon la revendication 1 ou 2, dans lequel :
la buse de raclage par gaz (1) comprend une pièce suspendue (3a) fixée à une surface supérieure de la cavité, la pièce suspendue (3a) n'atteignant pas une surface inférieure, et une pièce élevée (3b) fixée à la surface inférieure à une position espacée de la pièce suspendue (3a), la pièce élevée (3b) n'atteignant pas la surface supérieure ; et
le gaz introduit dans la passage d'écoulement de gaz à travers l'ouverture d'introduction de gaz (1e) est rectifié dans un procédé d'être circulé le long de la pièce suspendue (3a) et la pièce élevée (3b).

4. Dispositif de raclage par gaz selon l'une quelconque des revendications 1 à 3, dans lequel :
les éléments de blocage gauches et droits (2, 2) sont respectivement déplaçables par un mécanisme coulissant gauche (5A) et un mécanisme coulissant droit (5B), chacun étant un mécanisme coulissant distinct ;
le mécanisme coulissant gauche (5A) et le mécanisme coulissant droit (5B) sont montés sur une base commune (6), la base étant liée à un mécanisme coulissant (7) de base, et étant déplaçable ;
un capteur de position (4) pour détecter une position d'une bande d'acier est disposé à proximité de la sortie de gaz (1a) ;
le mécanisme coulissant gauche (5A) et le mécanisme coulissant droit (5B) sont configurés pour déplacer les éléments de blocage gauches et droits (2, 2) afin d'ajuster la largeur de la sortie de gaz ; et
le mécanisme coulissant de base (7) est configuré pour déplacer la base en accord avec des données de position de la bande d'acier détectées par le capteur de position (4), le déplacement de la base amenant le mécanisme coulissant droit (5B) et le mécanisme coulissant gauche (5A) à se déplacer, ainsi amenant les éléments de blocage gauches et droits (2, 2) à se déplacer, tout en maintenant la largeur de la sortie de gaz déjà ajustée.

5. Dispositif de raclage par gaz selon l'une quelconque des revendications 1 à 3, dans lequel :
les éléments de blocage gauches et droits (2, 2) sont respectivement déplaçables par un mécanisme coulissant gauche (5A) et un mécanisme coulissant droit (5B), chacun étant un mécanisme coulissant distinct ;
un capteur de position (4) pour détecter une position d'une bande d'acier est disposé à proximité de la sortie de gaz (1a) ;
le mécanisme coulissant gauche (5A) et le mécanisme coulissant droit (5B) sont configurés pour déplacer les éléments de blocage gauches et droits (2, 2) afin d'ajuster la largeur de la sortie de gaz ; et
le mécanisme coulissant gauche (5A) et le mécanisme coulissant droit (5B) sont configurés pour déplacer les éléments de blocage gauches et droits (2, 2) en accord avec des données de position de la bande d'acier détectées par le capteur de position, tout en maintenant la largeur de la sortie de gaz déjà ajustée.
